

Aug. 10, 1926.

1,595,866

W. S. LAWRENCE

TRANSFER SHEET AND METHOD OF MAKING SAME

Filed Sept. 17, 1924



INVENTOR  
Wentworth Lawrence  
BY  
M. H. Plum  
ATTORNEY

## UNITED STATES PATENT OFFICE.

WINTHROP STANLEY LAWRENCE, OF BROOKLYN, NEW YORK, ASSIGNOR TO KAUMA-  
GRAPH COMPANY, OF NEW YORK, N. Y., A CORPORATION OF NEW YORK.

## TRANSFER SHEET AND METHOD OF MAKING SAME.

Application filed September 17, 1924. Serial No. 738,136.

My invention relates to a new and improved transfer sheet and a new and improved method of making the same.

One of the objects of my invention is to provide a new and improved transfer sheet in which the transfer will be printed upon the paper forming the backing or base of the transfer, with the use of the ordinary reversed type now employed by printers, with a minimum of expense and without the need of making any special type for this purpose.

Another object of my invention is to provide a new and improved method of making a transfer sheet whereby the proper registration of the transfer marking upon the article upon which the transfer is to be made can be facilitated.

Another object of my invention is to provide a new and improved transfer sheet which will secure quick and accurate registration of the transfer marking upon the article upon which the transfer is to be made.

Other objects of my invention will be set forth in the following description and drawings which illustrate the preferred embodiment thereof, it being understood that the above statement of the objects of my invention is intended as a general explanation thereof, and not as a limitation thereof.

Fig. 1 diagrammatically shows the apparatus used for carrying out my method.

Fig. 2 shows the top of the transfer sheet formed by my new and improved method.

Fig. 3 shows the reverse of the said transfer sheet.

My invention is particularly directed to that type of transfer in which the marking is made upon a paper base, and the transfer marking is adapted to be released from the base when heat and pressure are applied. Of course, any equivalent material could be used for said paper base. Such transfers are very useful for marking linens and other fabrics, leather, etc. The ordinary printer's type is reversed so that it prints directly upon the paper. For the purposes of this specification, it may be stated that the transfer marking is first formed upon the type in reverse, is then printed on a tympan so as to be direct, is then reprinted by the tympan on the bottom of the transfer base in reverse, and after the transfer is completed is impressed directly on the article to be marked.

The base of the transfer ink, which may be any suitable indelible printing ink containing fast colors and no substances soluble in water, is applied upon the type 3 in the ordinary manner. In the first movement of the type 3, which may be of the ordinary and regular kind, the printing does not take place upon the paper base 2 of the transfer, but instead an imprint is made upon the tympan 1 which may be made of any suitable material such as paper or the like, so that the impression or marking made by the type 3, which is coated with the ink in any suitable manner, remains upon the surface of the tympan 1. At the next movement of the type 3, the paper 2 is inserted in the usual manner so that an imprint is simultaneously formed upon both sides of the paper, the said imprints being in exact registration with each other. The direct imprint 4 upon the top of the base can be read in the ordinary manner and this serves as a guide for transferring the reverse printing 5 upon the bottom of the paper, to the article, fabric, leather and the like upon which the transfer is to be made. This method permits the use of ordinary reverse type. Otherwise, it would be necessary to make special type.

After the imprint 5 has been formed upon the rear of the paper 2, it is dusted with a finely powdered composition while the ink is wet, so that this composition clings to the moist ink of the imprint 5, while the excess can be removed from the paper 2 by tapping the said paper. By this method this composition clings only to the lines of the imprint 5, after it has been fused and allowed to set.

Various powdered compositions can be used dependent upon the size of the type employed, but for 12 to 36 point type a suitable powdered composition may include the following:—

Dyestuffs soluble in oil such as indulines including the nigrosines, Victoria blue B base, oil red, which is a red dye basic in nature and soluble in mineral oil, can be incorporated in compositions containing a neutral resin such as paracoumarone resin with pigments which are resistant to alkaline washing fluids. Substances which as alpha nitro-naphthalene can be added to give increased stability and resistance to

the washing fluid whereby the dye which has been used has an affinity for the fibre of the fabric on which the impression is made

When certain dyes are used, as Victoria blue B base, the slow decomposition or removal of the carrying medium of the ink on washing causes the dye or pigment to become fixed in the fibre so as to produce a very permanent mark.

10 As a practical working example of such a composition, the following may be used, the proportions being by weight:

80 parts of paracoumarone resin such as "Cumar," 20 parts of a fast lithographic ink 15 having a blue color for example, 5 parts of a mineral oil having a specific gravity of 0.800, and 5 parts of Victoria blue B base.

I have found it highly desirable that the dusting composition should not consist of 20 resin alone but should also include viscous and liquid substances. For example, the lithographic ink above mentioned consists substantially of dried or thickened linseed oil, which is a viscous substance, and the mineral oil above mentioned is a liquid.

By mixing the relatively hard resin with a softer substance or substances, a fusible composition is formed which, when powdered to the proper degree of fineness, clings 30 to the moist ink impression so as to form a sharply defined design. I have also found that the proper admixture of the dyestuff or coloring substance with the resin is facilitated by the presence of the softer substance 35 or substances.

For type of 12-36 pt. the powder should go through a No. 9 sieve, but not through a No. 15 bolting cloth sieve. If the particles of the powder are too fine, then only a very 40 thin layer thereof clings to the ink.

Another example for giving a red impression would have the same proportions as above, save that the five parts of the Victoria blue B base are replaced by five parts 45 of the oil red before mentioned, and the five parts of mineral oil are replaced by five parts of a nitro-naphthalene, preferably alpha nitro-naphthalene.

Other pigments and dyestuffs could be 50 used to give colors other than red or blue. Of course, if pigments and dyestuffs are omitted from the dusting composition, a clear and colorless fused layer is formed upon the printing ink, which as before mentioned may be any suitable indelible printing ink containing fast colors and no substances soluble in water.

A large number of different formulae can be employed for the ink and for the dusting 60 composition employed in this method to meet various atmospheric and weather conditions and for the kind of work for which the transfer is intended. For example, the melting point can be adjusted by varying the 65 quantities of the softer elements of the be-

fore mentioned compositions such as the nitro-naphthalene, the mineral oil, the lithographic ink, etc.

When the reverse imprint on the paper 2 has been allowed to set after fusing, a raised 70 and fusible reverse imprint is formed, and the transfer can then be made in the ordinary manner by allowing the reverse imprint to come in contact with the article and then applying heat and pressure upon the 75 top of the transfer by a suitable heated iron or the like.

The transfer is formed upon the article to be marked in exact registration with the direct imprint upon the top of the paper. 80

It is desirable to gently heat the reverse imprint after the dusting composition has been applied thereto, and the excess has been removed, so as to fuse the powder thus retaining it in position upon the imprint or 85 impression on the paper.

In making transfers, it has been heretofore customary to print the paper with a fusible ink. It has also been suggested to print a sheet of paper provided with a fusible wax 90 coating with an ordinary non-fusible ink, and to then add a resinous ingredient to the said ink, so that the said ink would absorb this ingredient and become fusible. According to this invention, ordinary unwaxed 95 paper is printed with ordinary type and ink in the well known manner, and a raised fused surface layer of a fusible transfer ink composition is then formed on the marking formed with the ordinary ink. This surface 100 layer is so brittle that it could not be used by directly applying it to the paper by the ordinary intaglio printing process used in connection with ordinary fusible transfer inks. A transfer made as before specified 105

can therefore be manufactured very quickly and cheaply and without the use of intaglio printing cylinders. Experience has shown that the fusing of the powder causes it to intermix with the ink to a certain extent, which is an additional advantage. When the transfer is dusted with the powder, and the surplus powder is removed, the impression is somewhat ragged at the edges 110 due to adhering loose particles of the powder at the edges of the ink impressions. However, after the transfer has been heated, the lines of the impression become smooth, showing that the powder has been fused and has become intermixed with the ink so that 115 the outline of the transfer has the necessary smoothness. It is only necessary to heat a transfer for a few seconds in order to accomplish the fusing of the powder. The transfer can then be directly shipped, although it may be allowed to stand for a few 120 hours before shipment.

I have described a preferred embodiment of my invention but it is clear that numerous changes and omissions could be made with- 125

out departing from the spirit thereof and I do not wish to be limited to the details before specified.

I claim:-

- 5 1. A transfer comprising a paper base having a marking formed thereon with ink, the said marking having a fused non-tacky surface coating comprising a resin and a viscous substance, the said surface coating being substantially colorless and transparent.
- 10 2. A transfer comprising a paper base hav-

ing a marking formed thereon with ink, the said marking having a fused surface coating comprising a resin and linseed oil.

- 15 3. A transfer comprising a paper base having a marking formed thereon with ink, the said marking having a fused surface coating, the said surface coating including a resin, a viscous substance and a liquid.

In testimony whereof I hereunto affix my <sup>20</sup> signature.

WINTHROP STANLEY LAWRENCE.